

# UNITED STATES PATENT OFFICE.

FREDERICK WILLIAM WEEKS, OF EDGWORTH, ENGLAND.

## FIXATION OF ACID COLORS ON COTTON.

1,213,045.

Specification of Letters Patent. Patented Jan. 16, 1917.

No Drawing.

Application filed August 12, 1916. Serial No. 114,622.

To all whom it may concern:

Be it known that I, FREDERICK WILLIAM WEEKS, a British subject, residing at Edgworth, county of Lancaster, England, have 5 invented certain new and useful Improvements in the Fixation of Acid Colors on Cotton, of which the following is a specification.

This invention relates to improvements in 10 the fixation of acid colors on cotton in dyeing and calico printing.

Great efforts have been made to utilize 15 the acid wool colors in cotton dyeing and calico printing to give resulting shades which should be reasonably fast to washing and soaping. The usual methods of applying the aforesaid class of coloring matters to cotton fabrics, result in the production of shades which are extremely loose to washing and 20 materials so treated will not stand the slightest subsequent treatment such as washing or soaping.

The object of the present invention is to 25 produce dyed or printed shades on cotton goods, by means of the acid wool dyestuffs, which shall be capable of withstanding such after-treatment as is usually applied to dyed and printed goods produced by methods 30 commonly in use. Such after-treatment might be in the case of printed goods, a run through hot soap solution on the open soaping machine; or in the case of dyed goods a thorough washing with boiling water. To 35 produce such effects I utilize as fixing agents or mordants for the acid dyestuffs, the condensation products formed by the interaction of amines and aldehydes or their chemical equivalents.

In the production of dyed goods I impregnate 40 the material on the ordinary slop padding machine with a mixture made up as follows:— 12 ozs. anilin salt dissolved in 3 qts. water. To which when dissolved is added 1 pt. hexamethylene tetramin solution and the whole made up to 1 gallon. This padding mixture may have added to it, if desired, a small quantity of gum dragon thickening.

After padding and drying, the material 50 is mordanted and capable of being dyed with acid dyestuffs, using methods similar to those for applying the same dyestuffs to wool.

Another method of dyeing consists in 55 padding the material with a mixture containing the coloring matter and fixing agents

in the same bath. Thus a bright yellow may be dyed by padding the material in the following mixture.  $2\frac{1}{2}$  lbs. tartrazin dissolved in 8 gallons water, to which is added, 10 60 gallons gum dragon thickening 4 ozs. per gallon, 1 gallon anilin salt solution 4 lbs. per gallon, 1 gallon hexamethylene tetramin solution.

After padding and drying, fixation is 65 completed by steaming the goods 1 hour in a suitable steamer.

For printing we use colors made up on the following lines:— $7\frac{1}{2}$  lbs. Victoria scarlet 4R dissolved in 5 gallons water, to which is 70 added:— $4\frac{1}{2}$  lbs. maize starch.  $1\frac{1}{2}$  lbs. tapioca flour. The mixture is boiled well, cooled, and has added to it 7 lbs. gum dragon paste (4 ozs. per gallon), 3 gallons anilin salt solution (4 lbs. per gallon),  $2\frac{1}{2}$  75 gallons hexamethylene tetramin solution.

After printing and drying the material is steamed for 1 hour in a suitable steamer, after which it can be soaped and dried on the open soaping range.

In these examples the hexamethylene tetramin solution is prepared by mixing together equal volumes of ammonia 20% and formaldehyde 40%.

In practice it is found preferable to keep 85 the proportion of hexamethylene tetramin constant, as fixed in the previous recipe, and to vary the amount of anilin salt solution according to the color used, it being readily understood that such alteration is necessary, 90 owing to the great differences in constitution existing between the different members of the group of acid colors.

Although in the various examples given 95 the amine employed is a primary amine, viz., anilin salt solution the invention is not limited to primary amines but other amines will form compounds by their interaction with aldehydes which can be employed as the fixing agents or mordants.

It has been found that in the case of dyestuffs belonging to the series of sulfonated basic colors, *e. g.*, acid violet 2B, acid green, acid magenta, the reducing action of the formaldehyde comes into play during the 105 steaming operation, so that the shades produced require a suitable oxidizing process in order to develop them to their fullest intensity.

What I claim as my invention and desire 110 to protect by Letters Patent is:—

1. In the dyeing or printing of cotton fab-

- rics with acid dyestuffs, the method of treating the fabrics with fixing agents or mordants consisting of condensation products formed by the interaction of amines and aldehydes.
2. In the dyeing or printing of cotton fabrics with acid dyestuffs, the method of treating the fabric with fixing agents or mordants consisting of condensation products formed by the interaction of amines and aldehydes which yield an aldehyde when steamed or heated.
3. In the dyeing of cotton fabrics with

acid dyestuffs, the method of treating the fabric with fixing agents or mordants formed by the interaction of amines and aldehydes, the materials for forming said fixing agents or mordants being mixed in the padding bath with the acid dyestuffs.

In testimony whereof I have hereunto set my hand in presence of two subscribing witnesses.

FREDERICK WILLIAM WEEKS.

Witnesses:

J. OWDEN O'BRIEN,  
GEO. H. O'BRIEN.